

# UNITED STATES PATENT OFFICE.

WILBUR B. DRIVER, OF NEWARK, NEW JERSEY.

## MATERIAL FOR ELECTRICAL RESISTANCES AND THE LIKE.

1,217,578.

Specification of Letters Patent. Patented Feb. 27, 1917.

No Drawing.

Application filed April 29, 1911. Serial No. 624,132.

*To all whom it may concern:*

Be it known that I, WILBUR B. DRIVER, a citizen of the United States of America, and a resident of Newark, New Jersey, have invented a new and useful Improvement in Materials for Electrical Resistances and the like, which invention is fully set forth in the following specification.

My invention relates to alloys intended especially for electrical resistances. The object of the invention is to produce alloys which can be readily soldered, and to produce alloys of a closer and more cohesive grain in such electrical resistances as now have a tendency toward a separation of the grains, under working, thereby to render commercially available certain resistance-alloys which are not at present commercially useful or usable, owing to their friability or tendency to break or separate during the process of rolling and drawing.

In this art, an alloy is regarded as suitable for an electrical-resistance element if it has an electrical resistance of thirty or more microhms per cubic centimeter.

I have discovered, by study and experiment, that tin can be used as an ingredient of such alloys to good advantage in securing the objects above set forth. The addition of a proper amount of tin gives to the particular alloy at least two most desirable and distinct qualities which it did not theretofore possess:

First, although copper-manganese, copper-manganese-aluminum, copper-nickel, copper-nickel-manganese, etc., alloys have been used for electrical resistance purposes, it has been found difficult to solder in a permanent manner most if not all of these alloys. By the addition of a proper amount of tin, this difficulty can be and is to a great extent overcome. With reference to the proper amount of tin to be used in a particular composition (e. g., one wherein copper and manganese forms the body of the alloy), I have found about five (5) per cent. of tin to be very efficient, though less may be employed with some benefit, and a larger percentage can be used if desired. For instance, an alloy of copper 83%, manganese 12%, and tin 5%, gives a high electrical-resistance, a low temperature-coefficient, a low thermo-electric effect against copper, and good solderable quality.

Second, in some alloys, particularly those employing nickel and manganese (e. g., copper-nickel-manganese) the grains of the composition are in themselves often strong and tough, but there is little cohesion between the grains, and the alloy as a whole is not sufficiently strong and ductile to withstand rolling and drawing. For rendering such alloys workable, less tin is required than for rendering them capable of being soldered. I have found that the addition thereto of from one per cent. to two per cent. of tin, produces a marked improvement in ductility and cohesion and permits the working to be carried on to a greater extent and with more satisfactory results. But, if it is desired to render the alloy both workable and capable of being soldered a larger amount than from one to two per cent. of tin may be used.

The percentages above set forth are given merely as examples of the amount of tin which may be used to advantage in particular cases, but my invention is not limited to such percentages, and the amount of tin used can be varied to a considerable degree without departing from the spirit of my invention and the scope of its usefulness.

Having thus described my invention, I claim:

1. An electrical-resistance element consisting of an alloy containing copper and manganese, and having about five per cent. (5%) of tin.

2. An electrical-resistance element consisting of an alloy containing copper and some other ingredient, and having about five per cent. (5%) of tin.

3. An electrical-resistance element consisting of an alloy containing about five per cent. (5%) of tin.

4. An electrical-resistance element consisting of an alloy containing copper and at least five per cent. (5%) of manganese and about five per cent. (5%) of tin.

5. An electrical-resistance element consisting of an alloy containing copper and at least five per cent. (5%) of manganese and over four per cent. (4%) of tin.

6. An electrical-resistance element consisting of an alloy containing copper and at least five per cent. (5%) of manganese and over three per cent. (3%) of tin.

7. An electrical-resistance element consist-

ing of an alloy containing copper and at least five per cent. (5%) of manganese and over two per cent. (2%) of tin.

8. An electrical-resistance element consisting of an alloy containing copper and at least five per cent. (5%) of manganese and over one per cent. (1%) of tin.

In testimony whereof I have signed this specification in the presence of two subscribing witnesses.

WILBUR B. DRIVER.

Witnesses:

C. A. L. MASSIE,  
RALPH L. SCOTT.